

## UNITED STATES PATENT OFFICE

2,057,272

METHOD OF STRIPPING RHODIUM  
PLATING

Karl Schumpelt, Union, N. J., assignor to  
Baker & Company, Inc., a corporation of New  
Jersey

No Drawing. Original application April 20, 1935,  
Serial No. 17,390. Divided and this application  
May 12, 1936, Serial No. 79,270

13 Claims. (Cl. 75—101)

This application is a division of my copending application Serial No. 17,390, filed April 20, 1935.

The use of electrodeposited rhodium for protecting silverware, jewelry or silver plated articles against tarnishing and scratching, or for producing a pleasing white and lustrous finish on certain metals such as stainless steel, has become popular and extensive. However, it is desirable in some cases to remove the rhodium plating, especially from silverware and other articles formed of or plated with silver, for various reasons.

Various attempts have been made to remove the rhodium plating, for example, electrolytically by placing the article as the anode in acid solution, but the rhodium is so resistant to the action of acids that the silver or other metal of which the article is formed is injured or destroyed by the chemicals that have been used, so that such methods are impracticable. Therefore, it has been the general practice to remove the rhodium by grinding the rhodium plating from the article. This is a slow, laborious and expensive process, and great care and skill are necessary to prevent damage to the article. Therefore a prime object of my invention is to provide a novel and improved practical, easy and inexpensive method of removing the rhodium plating without injuring the article.

Generally, in electrodepositing rhodium for the purpose above-mentioned, it has been found desirable to electrodeposit a layer of nickel on the article preliminary to applying the finish layer of rhodium so that the rhodium is deposited on the nickel and a composite coating of nickel and rhodium results, and I contemplate the removing of rhodium plating by simply immersing the article in a solution containing an acid which will dissolve the nickel but which will not materially attack the metal of which the article is formed, for example silver. Also I contemplate forming on the surface of the article during the treatment thereof in the acid, a coating that will protect the metal of the article from attack by the acid regardless of the length of time that the article may remain in the acid. My method obviates the use of electric current and is inexpensive and safe in operation.

According to the present invention the method of stripping a composite coating formed of a plurality of layers of different metals from a silver or silver plated article, wherein the outer layer consists in or comprises one or more of the metals of the platinum group and the undercoating is formed of base metal, is characterized by

treating said coated article with a solvent that will dissolve the base metal but will not attack the metal of the article or the outer coating of the layer, particularly a bath including hydrochloric acid and water wherein the acid predominates. Thus, in accordance with the invention the method of stripping a composite coating of a plurality of layers of nickel or rhodium from silver or silver plated article wherein the nickel layer or layers constitute underplating for the rhodium, comprises the immersion of the coated article in an acid bath comprising hydrochloric acid or acetic acid or both, and water, which bath will dissolve the nickel but will not attack the silver.

More specifically describing the invention, especially for removing a composite coating of nickel and rhodium from a silver or silver plated article, the solution I prefer to use consists essentially of hydrochloric acid and water, although it is desirable to add a small quantity of aluminum sulphate to introduce the sulphate ion, and also to add a small quantity of sodium chloride to form a coating on the silver to protect the silver against attack from the acid. The formula in detail is

|                               |          |
|-------------------------------|----------|
| Hydrochloric acid.....        | 600 cc.  |
| Water.....                    | 400 cc.  |
| Aluminum sulphate, about..... | 30 grams |
| Sodium chloride, about.....   | 30 grams |

So far only inorganic acids which do not seriously attack silver have been specifically mentioned, although some organic acids which do not attack silver, such as acetic acid, may be used. Also acetic acid may be combined with hydrochloric acid as follows:

|                        |          |
|------------------------|----------|
| Hydrochloric acid..... | 500 cc.  |
| Acetic acid.....       | 200 cc.  |
| Water.....             | 300 cc.  |
| Sodium chloride.....   | 30 grams |

In all of the formulae, the proportions of the components are not critical and may be widely varied.

The method is carried out at a temperature 45 preferably ranging from 30 degrees C. to 70 degrees C., and the time required for completion of the method depends upon the amount of the electrodeposited metal. The article being treated is permitted to remain in the solution until the 50 nickel has been dissolved and the rhodium flakes off. The silver in the article is not damaged even where the article has engine turned surfaces, and in fact the silver is protected against injury by a coating for example of silver chloride 55

even upon prolonged immersion of the article in the solution.

The sodium chloride may be omitted where hydrochloric acid is present; and aluminum sulphate may be omitted although its presence is desirable. Furthermore, other metal sulphates such as ferric sulphate may be substituted for the aluminum sulphate.

In all cases the acid does not attack or affect 10 the rhodium, but I have found that the acid solution permeates the rhodium coating which is usually extremely thin and then dissolves the layer of nickel beneath the rhodium. The removal of the nickel of course frees the rhodium 15 from both the article and the nickel whereby the rhodium can be easily recovered.

After the nickel and rhodium have been removed from the article, the surfaces of the article can be easily polished.

20 Having thus described my invention, what I claim is:

1. The method of stripping a composite coating of a plurality of layers of nickel and rhodium from a silver or silver plated article wherein 25 the nickel layer or layers constitute underplating for the rhodium, said method consisting in immersing the coated article in a bath comprising hydrochloric acid, water and small quantities of a metal sulphate and sodium chloride.

30 2. The method of stripping a composite coating of a plurality of layers of nickel and rhodium from a silver or silver plated article wherein the nickel layer or layers constitute underplating for the rhodium, said method consisting in immersing 35 the coated article in a bath comprising hydrochloric acid, acetic acid, water, and a small quantity of sodium chloride.

3. The method of stripping a composite coating 40 of a plurality of layers of different metals from a silver or silver plated article wherein the outer layer comprises one or more metals of the platinum group and the inner layer or layers is formed of base metal, consisting in immersing the article with the coating in hydrochloric acid, 45 water and small quantities of a metal sulphate.

4. The method of stripping a composite coating 50 of a plurality of layers of different metals from a silver or silver plated article wherein the outer layer comprises one or more metals of the platinum group and the inner layer or layers is formed of base metal, consisting in immersing the article with the coating in a bath comprising 55 hydrochloric acid, acetic acid, water, and a small quantity of sodium chloride.

5. The method of stripping a composite coating 60 of a plurality of layers of nickel and rhodium from a silver or silver plated article wherein the nickel layer or layers constitute underplating for the rhodium, said method consisting in immersing the coated article in a bath comprising a mixture of hydrochloric acid and water wherein hydrochloric acid is the major portion.

6. The method of stripping a composite coating 65 of a plurality of layers of nickel and rhodium from a silver or silver plated article wherein the nickel layer or layers constitute underplating for the rhodium, said method consisting in immersing the coated article in a bath comprising a mix-

ture of hydrochloric acid and water wherein hydrochloric acid is the major portion and a small quantity of a metal sulphate.

7. The method of stripping a composite coating 5 of a plurality of layers of nickel and rhodium from a silver or silver plated article wherein the nickel layer or layers constitute underplating for the rhodium, said method consisting in immersing the coated article in a bath comprising a mixture 10 of hydrochloric acid and water wherein hydrochloric acid is the major portion and a small quantity of aluminum sulphate.

8. The method of stripping a composite coating 15 of a plurality of layers of nickel and rhodium from a silver or silver plated article wherein the nickel layer or layers constitute underplating for the rhodium and said method consisting in immersing the coated article in a bath comprising a mixture of hydrochloric acid and water in the proportions of three-fifths of a liter of hydrochloric acid and two-fifths of a liter of water.

9. The method of stripping a composite coating 25 of a plurality of layers of nickel and rhodium from a silver or silver plated article wherein the nickel layer or layers constitute underplating for the rhodium and said method consisting in immersing the coated article in a bath comprising a mixture of hydrochloric acid and water in the proportions of three-fifths of a liter of hydrochloric acid and two-fifths of a liter of water and 30 about 30 grams of aluminum sulphate.

10. The method of stripping a composite coating 35 of a plurality of layers of nickel and rhodium from a silver or silver plated article wherein the nickel layer or layers constitute underplating for the rhodium, said method consisting in immersing the coated article in a bath comprising a mixture of hydrochloric acid and water wherein hydrochloric acid is the major portion, and acetic 40 acid.

11. The method of stripping a composite coating 45 of a plurality of layers of nickel and rhodium from a silver or silver plated article wherein the nickel layer or layers constitute underplating for the rhodium, said method consisting in immersing the coated article in a bath comprising a mixture of hydrochloric acid and water wherein hydrochloric acid is the major portion, and an organic acid that will not attack silver.

12. The method of stripping a composite coating 50 of a plurality of layers of nickel and rhodium from a silver or silver plated article wherein the nickel layer or layers constitute underplating for the rhodium and said method consisting in immersing the coated article in a bath comprising 55 a mixture of hydrochloric acid and water in the proportions of about one-half liter of hydrochloric acid, about one-third liter of water, and about one-fifth liter of acetic acid.

13. The method of stripping a composite coating 60 of a plurality of layers of different metals from a silver or silver plated article wherein the outer layer comprises one or more metals of the platinum group and the inner layer or layers is formed of base metal, said method consisting 65 in immersing the coated article in a bath comprising a mixture of hydrochloric acid and water wherein hydrochloric acid is the major portion.

KARL SCHUMPELT.